

I. A. BRADDOCK.  
PROCESS OF TREATING ORES.  
APPLICATION FILED JUNE 18, 1910.

987,850.

Patented Mar. 28, 1911.



# UNITED STATES PATENT OFFICE.

ISAAC A. BRADDOCK, OF HADDONFIELD, NEW JERSEY, ASSIGNOR OF ONE-SIXTH TO WILLIAM C. CODD, OF BALTIMORE, MARYLAND, AND ONE-SIXTH TO NICHOLAS A. KESTLER AND ONE-SIXTH TO DAVID E. ANTHONY, OF WASHINGTON, DISTRICT OF COLUMBIA.

## PROCESS OF TREATING ORES.

987,850.

Specification of Letters Patent. Patented Mar. 28, 1911.

Application filed June 18, 1910. Serial No. 567,573.

*To all whom it may concern:*

Be it known that I, ISAAC A. BRADDOCK, residing at Haddonfield, in the county of Camden and State of New Jersey, have invented certain new and useful Improvements in Processes of Treating Ores, of which the following is a specification.

My invention is an improved process for treating metalliferous ores, particularly those bearing the more valuable metals, such as gold, silver, copper, etc., and in its generic nature the invention resides in taking uncrushed ores as they come from the mines or after they have passed through the primary breakers and alternately lifting and dropping the same onto a hard surface or surfaces within a container whereby to pulverize the ores, and while dropping subjecting such ores to a high temperature by dry heat to drive off the water of crystallization and volatile products in the ore and render the ore mass spongy and cause the same to decrepitate, thereby assisting in breaking and crushing the ore on impacting 25 with the hard breaker body so as to pulverize the ore.

My invention also consists in providing a process wherein crushed and finely divided ore is separated from the coarser uncrushed ore and delivered while hot into a suitable bath for further treatment and acting on the hot pulverized ore stream prior to its deliverance into the bath to reduce its temperature an amount sufficient to maintain a constant or practically constant temperature of bath.

My process also includes the simultaneous dry heating and crushing of the ores to produce a hot dry powder and then delivering the same while hot into a bath of suitable material for the separation of the ore values, without introducing steam or water to the ores prior to their introduction into the solvent or bath.

The apparatus I prefer to employ in carrying out my process forms the subject-matter of a copending application, filed on even date herewith, Serial No. 567,572, and

is briefly indicated in the drawings forming part of this application in which:

Figure 1, is a central vertical longitudinal section of the preferred form of apparatus. Fig. 2, is a cross section on the line 2—2 of Fig. 1. Fig. 3, is a central vertical longitudinal section of a slightly modified form of apparatus.

The apparatus I prefer to employ to carry out my invention consists briefly of a first container 1 of globular form, slightly elongated and provided with hemispherical ends through one of which the ores and hot blast are introduced and through the other of which the treated ore is delivered. This container 1 is in its preferred construction composed of a metal frame-work 2 embedded in a fire-proof substance 3, such as concrete, clay or the like, and lined with a crusher lining 4 of rocks of a suitable material. The second container 6 is of substantially the same construction and contains the solvent 7. The first container 1 has an inlet 8 and an outlet 9 through the hemispherical ends, the outlet 9 delivering into the inlet 10 of the container 6, whose outlet 11 is directly opposite.

12 designates partitions within the container 1, and 13 designates the partitions within the container 6. These partitions are radial and terminate short of the central axis of the containers to produce an uninterrupted central longitudinal passage 14 from the entrant end 8 of one container to the exit end 11 of the other container. A suitable hot blast 15 is provided within the container 1 from substantially the entrant end 8 to the exit end 9 in the central zone 14. This blast may be produced by an oil burner 16 or by a blower 17, when hot fuel 18 is used, a grate or table 19 being provided, by means of which the ore and fuel may be introduced into the container 1 when hot fuel is used.

The containers 1 and 6 are supported on suitable cradles formed of rollers 20 mounted in supports 21 and the containers are turned by rollers 22 on a shaft 23 to which

motion is imparted by a belt 24 and pulley 25. It will be noticed that the entrant end 10 and exit end 11 of the containers 6 and 1 respectively are in close juxtaposition to one another and are slightly separated to form an air inlet 26 whose area may be adjusted by a collar 27, for a purpose hereinafter explained. The solvent 7 may be admitted to the container 6 in any desired manner, preferably by a pipe 28, as shown in the drawings.

The ore 29 to be treated is placed in the container 1 and the fuel for heating is also introduced when the oil burner 16 is used 15 to produce the heat blast from inlet to outlet of the container 1. I prefer to use one that will produce a blast somewhat of the type shown in the drawings. Having introduced the ore in large chunks as it comes from the 20 mine (or after it has passed through the first breakers) into the container 1 and having introduced the solvent into the container 6 (the solvent being a cyanid or other solution when gold and silver ores are undergoing treatment) a hot blast is produced 25 by igniting the burner 16 in any desired manner, and the containers are set in motion. The ore 29 will be carried up by the partitions 12 and 13 and dropped through the 30 blast or flame 15 where they will come into direct contact with the hot blast and have their water of crystallization and volatile products driven off. Any sulfur in the ore will be removed in this manner. The ore 35 having dropped through the hot blast 15 impacts the crusher surface 4 of the container at the bottom and inasmuch as the structure of the ore in being heated is weakened and made porous, the impact will 40 break and crush the ore, which breaking and crushing is further assisted by the rolling and tumbling of the softer particles in connection with the harder particles in the container 1 during its rotation. The temper- 45 ature within the container 1 is usually carried up to about 500° F. so as to thoroughly dry the ore and drive off the volatile products.

Attention is called to the fact that the 50 removal of the volatile products in the ore while passing through the heat zone causes decrepitation to take place, and the ore becomes porous and spongy so when it contacts the bottom of the container it will be 55 broken and crumbled, the breaking and crumbling action being also assisted by the rolling and tumbling of the ore within the retort during its movements, the heavier and lesser heated ores serving to assist in 60 crushing the softer particles until the ore is reduced to a fine powder. The force of the heated blast serves to cause the crushed particles of the ore to gradually work toward the outlet 9 of the container and as soon as 65 the ore rocks have been crushed fine enough

the heated blast will carry the ore particles through the outlet 9 of the retort 1 into the second container 6 where the hot ore particles are deposited into the solvent 7. The container 6 being provided with partitions 13 will serve to agitate the solution within the container 6 and as the hot ore particles are directly deposited into said solution the temperature within the container 6 will be maintained at the desired degree (usually 75 from 200° to 212° F.) The air opening between the containers 1 and 6 is so regulated that the temperature within the container 6 will be maintained constant or practically so, so as to avoid the boiling of the solvent 80 but still allow sufficient heat to assist the chemical re-action.

As soon as a sufficient quantity of ore is deposited in the solution 7 in the container 6, said container is rolled away and another 85 container substituted. The dissolved ore and solvent from the container 6 which has been rolled away may be emptied after forced percolation by steam or vacuum, or both, and extracting the values thereby into 90 any suitable reservoir where it may be further treated by the usual means to separate the dissolved values if any remain.

Having thus described the process and the preferred form of apparatus, I call attention 95 to the fact that in lieu of using a gas burner 16, other fuel may be used as conditions warrant, and as will be more clearly apparent by reference to my copending application hereinbefore referred to.

In this application I make no claim to the apparatus as such as that forms the subject-matter of my other application hereinbefore referred to, and I further desire to state that slight changes in the sequence of 105 steps of my process herein described, or slight modifications in the various degrees of temperature used may be made dependent upon the ore being treated and as will be apparent to those skilled in the art, without 110 departing from the spirit of the invention, or the scope of the appended claims.

What I claim is:

1. The process of treating ores which consists in placing a body of ore within a tubular container, establishing a hot blast through said container, successively lifting said ore above said blast and then dropping it through said blast upon the bottom of said container to pulverize said ore, and finally removing the pulverized ore from the container by said blast.

2. The method of treating ores which consists in placing a body of ore in a container having an inlet and an outlet, establishing a hot blast from the inlet to the outlet to raise the temperature within said container to a definite degree, then successively lifting said ore above said blast and dropping it through said blast to become crushed and

115

120

125

130

5 pulverized until said ore has been sufficiently pulverized to be delivered out of said container by said blast, and causing said blast to deliver said ore out of said container into a second container containing a solvent and depositing said ore into said solvent.

3. The method of treating ores which consists in placing a body of ore in a container having an inlet and an outlet, establishing a 10 hot blast from the inlet to the outlet to raise the temperature within said container to a definite degree, then successively lifting said ore above said blast and dropping it through said blast to become crushed and pulverized 15 until said ore has been sufficiently pulverized to be delivered out of said container by said blast, and causing said blast to deliver said ore out of said container into a second container and retaining said ore so delivered in 20 said second container.

4. The method of treating ores which consists in placing a body of ore in a container having an inlet and an outlet, establishing a hot blast from the inlet to the outlet to 25 raise the temperature within said container to a definite degree, then successively lifting said ore above said blast and dropping it through said blast to become crushed and pulverized until said ore has been sufficiently 30 pulverized to be delivered out of said container by said blast, causing said blast to deliver said ore out of said container into a second container, retaining said ore so delivered in said second container, and subjecting the ore delivered into said second container to chemical action to separate the 35 values therefrom.

5. A process of treating ores consisting in introducing the ore into a container and 40 simultaneously heating, drying and pulverizing the ore in said container, and then delivering said ore while hot into a solvent.

6. A process of treating ores consisting in introducing the ores into a container and 45 simultaneously heating, drying and pulverizing the ore in said container, then delivering said ore while hot into a solvent, and cooling said ore prior to its delivery into said solvent, a sufficient amount to maintain 50 a constant temperature in the solvent.

7. A process of treating ores which consists in introducing ores into a container and subjecting them to the action of a hot dry blast to cause said ores to become porous and 55 decrepitate, dropping and tumbling said ores within said container while hot to crush the same, and then blowing the crushed ore particles out of said container into a second container for further treatment.

60 8. A process of treating ores which consists in introducing ores into a container and subjecting them to the action of a hot dry blast to cause said ores to become porous and decrepitate, dropping and tumbling said 65 ores within said container while hot to crush

the same, then blowing the crushed ore particles out of said container into a second container for further treatment, and then subjecting the ore so delivered to the action of a solvent.

70

9. A process of treating ores which consists in introducing ore chunks into a container, subjecting said ore to the action of a dry hot blast and simultaneously tumbling said ore to drive off the volatile products 75 thereof and pulverize said ore and then blowing said ore out of said container into a receptacle for further treatment.

10. A process of treating ores which consists in providing two containers each having an inlet and an outlet in alinement with one another, the inlet of one container being adjacent to the outlet of the other container, establishing a hot blast through said containers with a heating zone extending 80 from the inlet to the outlet of the first container, introducing ore chunks into said first container and then lifting said ore chunks and dropping them through said heat zone to render said ore chunks porous and cause 85 them to decrepitate and become pulverized on contact with the container wall until the ore becomes sufficiently pulverized and then convey said pulverized ore by said blast into said second container and preventing said 90 ore particles from leaving said second container.

11. A process of treating ores which consists in providing two containers each having an inlet and an outlet in alinement with 100 one another, the inlet of one container being adjacent to the outlet of the other container, establishing a hot blast through said containers with a heating zone extending from the inlet to the outlet of the first container, introducing ore chunks into said first container and then lifting said ore chunks and dropping them through said heat zone to render said ore chunks porous and cause 105 them to decrepitate and become pulverized on contact with the container wall until the ore becomes sufficiently pulverized and then convey said pulverized ore by said blast into said second container and preventing said 110 ore particles from leaving said second container, and subjecting said ore particles to further treatment in said second container to separate the values therefrom.

12. A process of treating ores which consists in providing two containers each having an inlet and an outlet in alinement with one another, the inlet of one container being adjacent to the outlet of the other container, establishing a hot blast through said containers with a heat zone extending from 120 the inlet to the outlet of the first container, introducing ore chunks into said first container and then lifting said ore chunks and dropping them through said heat zone to render said ore chunks porous and cause 125

130

them to decrepitate and become pulverized on contact with the container wall until the ore becomes sufficiently pulverized and then convey said pulverized ore by said blast into said second container and preventing said ore particles from leaving said second container, subjecting said ore particles to further treatment in said second container to

separate the values therefrom, while maintaining a constant temperature in said second container at a predetermined degree.

**ISAAC A. BRADDOCK.**

Witnesses:

DAVID E. ANTHONY,  
WM. S. ARMSTRONG, Jr.